

April 28, 1931.

F. SINGER

1,802,785

METHOD OF EXTRUDING LONG SEAMLESS TUBING

Filed Oct. 11, 1924



Fig. 1

Fig. 2



Fig. 3



Fig. 4



Inventor:

Ferd. Singer  
by *Ferd. Singer*  
Attorney

## UNITED STATES PATENT OFFICE

FRITZ SINGER, OF NUEREMBERG, GERMANY

## METHOD OF EXTRUDING LONG SEAMLESS TUBING

Application filed October 11, 1924. Serial No. 743,146.

The present invention relates to an improved heat extrusion process for the production of seamless tubes of perforated or imperforated billets of copper, zinc, aluminum and other metals and alloys which can be extruded above 300° C. and below 900° C.

In the manufacture of these tubes, the problem is to extrude large amounts of metals in a plastic condition through the ring-shaped opening between the mandrel and the die.

Heretofore, in heat extrusion of tubes the pressing surface of the punch has always been made flat and the surface of the die given only a slight bevel or inclination at most. It has now been found that the bevel angle of the die surface exerts considerable influence on the result, and that a bevel angle of about 27°, with a permissible deviation of a few degrees above and below, is the best and that greater deviations from this angle results in defects such, for example, as doubling, in the last extruded portions of the tube. These defects do not arise in heat extruded pipes in hydraulic presses, as a considerable press residue remains in the receiver.

In hydraulic heat extrusion the press residue amounts to 10-15% of the weight of the ingot, while it is possible with the use of a crank press to reduce it to 2-3% thereof. This result is to be ascribed on the one hand to the great increase of the pressure at the end of the stroke, and on the other to the inclined formation of the operative surfaces of the punch and the die, which permit the remainder of the ingot to flow out uniformly.

Referring now to the drawings in which like reference characters indicate corresponding parts throughout:

Figure 1 is a vertical longitudinal section through the extrusion tool, wherein the full lines show the position of the press punch at the beginning of the extrusion and the dotted lines the position thereof on termination of the perforating step,

Fig. 2 is a similar section through the extruding tool, showing the press punch in its lowermost position and the extruded tube,

Fig. 3 is a longitudinal section through a

metal ingot, which is partially perforated for guiding the perforating punch or mandrel,

Fig. 4 is a longitudinal section through a metal ingot provided with a perforation 55 through its entire length.

On top of the apertured bed-plate of an upright crank press (not shown on the drawing) the apertured base-plate *g*, the container *d* and the matrix die *f* are mounted together. The matrix die rests with the container on said base-plate and is surrounded by the container. The die *f* has a bore *f'* which corresponds to the outer diameter of the finished tube and extends into a large bore.

The conical face of the matrix die bearing the billet forms an angle of about 30° with the horizontal plane.

The punch *a* is mounted on the reciprocating member of the crank press (not shown in the figures) and provided at its lower end with an annular reinforcement *b*. The end of the punch is turned off on a bevel to agree accurately with the face of the matrix die.

The perforating mandrel *c* is attached to the punch. The billet *h* or *h'* is adapted to be inserted in the container. The billet *h* is partially, the billet *h'* totally bored, the partial hole *l* or the complete bore *l'* being adapted to guide the mandrel.

The process is carried out in the following manner:

The billet of metal to be extruded is heated to a suitable temperature and is then inserted in the container. The punch and mandrel which have been heated by a gas flame and coated with a friction material such as a mixture of oil and graphite will now descend and the mandrel will enter the hole *l* or the bore *l'*, depending upon the type of billet used. If the billet *h* is used the mandrel will be forced through the billet and into and through the die. This will cause the metal to ascend as indicated by the dotted lines *h'* and a portion of the metal will be forced through the die ahead of the mandrel as a plug *m* before the extrusion of the tube begins.

As soon as the punch contacts with the metal so that the metal can no longer ascend, it will be extruded through the an.

nular opening, between the die and the mandrel, to thereby form the tube *i* as shown in Fig. 2.

The entire quantity of metal making up the billet is extruded as a tube with the exception of the plug  $m$  and the thin-flared residue  $k$ , which is connected with the tube.

In order to remove the tube from the tool the residue  $k$  is cut off along the edge of the tube by means of a circular chisel, whereupon the tube drops down, the residue adhering to the chisel with which it is removed.

The working temperatures most suitable for the several metals and alloys are easily ascertained. For aluminium they are between  $350^{\circ}$  and  $450^{\circ}$  C., for brass alloys between  $650^{\circ}$  and  $800^{\circ}$  C. and for copper between  $800^{\circ}$  and  $900^{\circ}$  C.

I claim as my invention:

20. The method of extruding a long seamless tube from a large block of metal of greater length than diameter, comprising heating the block to a temperature of not less than about  $350^{\circ}$  C., and while in a container applying pressure to the thus-heated block in the direction of its length between relatively-moving members having concentric conical opposing block-engaging surfaces inclined at approximately  $60^{\circ}$  to the center line of said 25 pressure, thereby extruding all but a small residue of said block as a long seamless tube of uniform physical characteristics throughout.

In testimony whereof I affix my signature.  
FRITZ SINGER.

## 35. **FRITZ SINGER**

40. *Converso* é o termo usado para designar os  
que se converteram ao catolicismo, e que  
não eram católicos de origem. O termo  
é usado para designar os que se conver-  
tiram ao catolicismo, e que não eram  
católicos de origem.

45. *Indicates a deficiency of calcium in the diet. It is  
characterized by frequent convulsions, especially  
at night, and fits of spasmodic convulsions, and  
loss of consciousness. It is best treated by  
administering a 10 per cent. solution of calcium  
carbonate, and the administration of the same  
solution repeated at intervals of two hours.*

55  
56  
57  
58  
59  
60

60 *Journal of the American Revolution* 1 (2009)